

## UNITED STATES PATENT OFFICE

2,450,773

DYEING OF WOOL WITH INDIGO  
DYESTUFFSEdward Weber, Winchester, Mass., assignor to  
Allied Chemical & Dye Corporation, New York,  
N. Y., a corporation of New YorkNo Drawing. Application March 30, 1944,  
Serial No. 528,772

5. Claims. (Cl. 8—36)

1

This invention relates to the dyeing of animal fibers, and especially wool, with indigoid vat dyestuffs. It relates more particularly to an improved method of exhausting an ammonia-hydrosulfite vat of an indigoid vat dyestuff, or related dye liquor, employed in the dyeing of animal fibers.

The dyeing of animal fibers with indigoid vat dyestuffs, and especially indigo, presents a number of difficulties which ordinarily are not encountered in the dyeing of cotton and other vegetable fibers. Thus, because of the chemical nature of the animal fibers, it is necessary to avoid the use of strongly alkaline vats or related dye liquors. It has accordingly been the practice to dye woolen stock, yarn, slubbing, or piece-goods in a weakly alkaline vat, or with a circulating liquor, containing a leuco-compound of an indigoid vat dyestuff, aqueous sodium hydrosulfite and a weak alkali (such as ammonium hydroxide, sodium carbonate, or the like), and preferably also containing a dispersion assistant (such as a protective colloid or an organic dispersing agent; for example, glue, gelatin, synthetic organic compounds of the alkyl aryl sulfonate type, and the like).

Prior to the present invention, in the dyeing of animal fibers with indigoid vat dyestuffs, it was known to exhaust an ammonia-hydrosulfite vat of an indigoid vat dyestuff, or related dye liquor, by adding thereto ammonium sulfate or other acidic substance, such as an acid (e. g., hydrochloric acid, acetic acid, lactic acid, etc.) or an acid salt (e. g., ammonium chloride, ammonium formate, sodium bisulfite, etc.). It was also known, in the dyeing of vegetable fibers, to exhaust a sodium hydroxide-hydrosulfite vat or other strongly alkaline vat of an indigoid vat dyestuff by adding to the vat neutral sodium sulfate (e. g., Glauber's salt) or common salt. While the possibility of exhausting an ammonia-hydrosulfite vat with sodium sulfate was recognized by the prior art, it was rejected as unsuitable in view of the fact that sodium sulfate is a neutral salt, whereas for the dyeing of animal fibers it was considered necessary, prior to the present invention, to neutralize the vat by means of an acidic substance in order to exhaust it. (See, for example, American Dyestuff Reporter, vol. XIX, 1930, page 241.)

It has been discovered in accordance with the present invention that the neutral alkali metal sulfates and the alkali metal chlorides not only are effective as exhausting agents for ammonia-hydrosulfite vats in the dyeing of animal fibers

2

with indigoid vat dyestuffs, but in some cases produce superior dyeings. For example, in the dyeing of woolen piece-goods with indigo from an ammonia-hydrosulfite-glue vat, it has been found, in accordance with the present invention, if sodium sulfate (e. g., Glauber's salt) is added to the vat as an exhausting agent, the resulting dyeings are about 10% stronger than dyeings obtained under similar conditions with the same materials but with ammonium sulfate as the exhausting agent, and the dyeings are otherwise substantially identical.

Thus, in accordance with the present invention, dyeings which are of equal or greater tinctorial strength, as compared with those obtained with the use of ammonium sulfate, can be obtained without sacrificing any of the important qualities of the dyeings (especially uniformity, penetration, and fastness to crocking) by the use of such readily available and cheap salts as sodium sulfate and sodium chloride. (It will be understood that where sodium sulfate is referred to herein and in the claims, the neutral sulfate,  $\text{Na}_2\text{SO}_4$ , with or without water of crystallization, is intended.)

The neutral alkali-metal sulfate or alkali-metal chloride (for example, sodium sulfate, potassium sulfate, sodium chloride, potassium chloride, lithium chloride, etc.) is preferably added to the vat or other dye liquor in small amounts during the course of the dyeing, to effect a gradual precipitation of the leuco compound and thereby promote even dyeings characterized by good penetration and fastness to crocking. It is preferably added to the dye liquor after dyeing has progressed to a substantial degree, in accordance with the usual practice in the art in exhausting indigoid vat dyestuff liquors; it may be added earlier, however, if desired.

The invention will be illustrated by the following specific example, but it is to be understood that the invention is not limited to the details thereof and that changes may be made without departing from the scope of the invention.

## EXAMPLE

Eleven-ounce woolen piece-goods were processed and dyed in rope form in an ordinary piece-dye kettle (which machine) open to the atmosphere in the following manner, the ratio of the goods to the dyebath or liquor being always maintained at about 1:20. The amount of reagent used in each case is given in terms of 100 pounds of cloth.

*Washing*

The goods were first washed by circulating them for 30 minutes in a bath at 180° F. and composed of water, 2 lbs. of "Nacconol NR" (a commercial surface-active agent comprising a mixture of alkyl benzene sodium sulfonates derived from kerosene) and 4 lbs. of 26% ammonium hydroxide. The goods were then washed free from alkali with water.

*Bottoming with chrome dyes*

A dyebath was prepared by warming the water in the kettle to 110° F. and adding:

2 oz. of Alizarol Azurine ECA  
 3 lbs. 8 oz. of Superchrome Blue BC  
 1 lb. 3 oz. of Superchrome Blue B High Conc. (C. I. 202)  
 2 lbs. 8 oz. of Superchrome Red ECB  
 3 oz. of Superchrome Yellow RN (C. I. 197)  
 10 lbs. of calcined Glauber's salt (Na<sub>2</sub>SO<sub>4</sub>)  
 6 lbs. of 56% acetic acid.

The winch was set in motion, and the dyebath was heated to boiling during one hour. The bath was boiled for an additional hour and then cooled to 160° F. (by displacing part of the exhausted dyebath with cold water) at which point 3 lbs. of sodium bichromate, dissolved in water, were introduced. The bath was reheated to boiling during 15 minutes, and boiled for 45 minutes, after which it was displaced with water. The goods were rinsed until a clear rinse liquor was obtained.

*Topping with indigo*

A stock vat of indigo was prepared by pasting 10 lbs. of indigo NAC 20% Paste (Color Index 1177) with a solution of 1 lb. of caustic soda flakes in 5 lbs. of cold water, sprinkling in 1 lb. 11 oz. of sodium hydrosulfite powder, and heating the resulting mixture to 125° F. until reduction of the indigo to the leuco compound was complete.

A bath was prepared by adding to the water in the kettle:

6 lbs. of 26% ammonium hydroxide, 2 lbs. of animal glue, and 3 lbs. of sodium hydrosulfite. The resulting mixture was heated to 125° F. and the goods were circulated for 10 minutes. The stock vat of indigo was quickly added to the bath, and dyeing was carried out at 125° F. for 20 minutes. Then 10 lbs. of calcined Glauber's salt (Na<sub>2</sub>SO<sub>4</sub>), dissolved in 100 lbs. of water, were added slowly during 10 minutes to exhaust the dyebath. The goods were then rinsed and circulated through cold running water until the leuco-indigo was oxidized substantially completely.

The dyed goods thus obtained were scoured with soap in the conventional manner to remove loosely-held indigo, rinsed and dried.

The goods were dyed full and well-penetrated navy blue shades possessing good evenness (levelness) and fastness to crocking.

In the above examples, sodium sulfate is used as an exhausting agent for an ammonia-hydrosulfite-glue vat in connection with the dyeing of chrome-bottomed woolen piece-goods in rope form with indigo, which is claimed in my application Serial No. 528,711, filed March 20, 1944, now abandoned. The invention is not limited thereto, however.

Thus, the invention may be applied to the dyeing of wool which has not been predyed with another dyestuff; for example, it may be employed in the dyeing of carbonized or uncarbonized wool in an ammoniacal indigo vat.

Instead of sodium sulfate, another neutral alkali-metal sulfate or alkali-metal chloride or a mixture thereof may be employed as exhausting agent. The amount of exhausting agent which is required depends upon the conditions employed (e. g., amount of dye liquor, temperature, etc.) and can be easily determined in each case; for example, by slowly adding various amounts of the exhausting agent to the dye liquor, and noting the minimum amount of exhausting agent which produces dyeings of maximum tinctorial strength (corresponding for all practical purposes with optimum exhaustion of the dyebath). Thus, in the foregoing example, the use of substantially less than 10 pounds of sodium sulfate results in an incomplete exhaustion of the dyebath, while the addition of substantially more than 10 pounds of sodium sulfate does not noticeably improve the tinctorial strength of the dyeing. In general, at least 1/2 per cent of sodium sulfate, based on the weight of the dye liquor, or equivalent weight of another neutral alkali metal sulfate or an alkali metal-chloride, is required to effect substantially complete exhaustion of the dyebath.

The dye liquor need not contain glue; but preferably it contains a dispersion assistant (such as glue and/or another protective colloid or organic dispersing agent).

The invention includes the dyeing of proteinous fibers of various kinds, including natural animal fibers (such as wool, silk, hair and the like) and artificial animal fibers (such as those derived from casein, soybean and the like), all of which are comprehended within the generic term "animal fibers" herein and in the claims.

The invention may be employed in connection with dyeing of the animal fibers in various forms (e. g., stock, slubbing, yarn, piece-goods, etc.), by hand, in various types of dyebaths (including stationary and circulating dyebaths or liquors), and in various forms of apparatus.

Further, vats and dye liquors of other vat dyestuffs of the indigoid series may be exhausted by means of the exhausting agents of the present invention, as for example:

Vat Orange R \_\_\_\_\_ Color Index No. 1217  
 Vat Red Violet RH \_\_\_\_\_ Color Index No. 1212  
 Vat Pink FF \_\_\_\_\_ Am. Assoc. Textile  
 Chemists and Color-  
 50 ists, Vol. XIX (1942),  
 page 523.  
 Brilliant Indigo 4BR \_\_\_\_\_ Color Index No. 1184  
 Brilliant Indigo KMR \_\_\_\_\_ Color Index No. 1183

I claim:

1. In the dyeing of wool with an indigo by treating the wool with a dye liquor comprising an indigo in the leuco form, sodium hydrosulfite and ammonium hydroxide, the improvement which comprises exhausting the dye liquor by adding thereto an alkali-metal salt selected from the group consisting of the neutral alkali-metal sulfates and the alkali-metal chlorides.

2. In the dyeing of wool with indigo by treating the wool with a dye liquor comprising indigo in the leuco form, sodium hydrosulfite and ammonium hydroxide, the improvement which comprises exhausting the dye liquor by adding sodium sulfate thereto.

3. In the dyeing of wool with an indigo from an ammonia-hydrosulfite-glue vat, the improvement which comprises adding sodium sulfate to the vat in small amounts at a time, while continuing the dyeing, the total amount of sodium sulfate being at least sufficient to exhaust the vat substantially completely.

4. The method of dyeing wool with indigo which comprises subjecting wool to a dyeing treatment with a weakly alkaline dye liquor containing leuco-indigo, sodium hydrosulfite, ammonium hydroxide and an organic dispersing assistant, then adding sodium sulfate to the dye liquor, as an exhausting agent, and continuing the dyeing treatment.

5. The method of dyeing wool with indigo which comprises dyeing woolen piece-goods in a weakly alkaline vat containing leuco-indigo, sodium hydrosulfite, ammonium hydroxide and glue, and adding sodium sulfate to the vat in small amounts at a time, as an exhausting agent, while continuing the dyeing, the total amount of sodium sulfate being at least sufficient to exhaust the vat substantially completely.

EDWARD WEBER.

REFERENCES CITED

The following references are of record in the file of this patent:

UNITED STATES PATENTS

| Number    | Name     | Date           |
|-----------|----------|----------------|
| 972,066   | Deinet   | Oct. 4, 1910   |
| 1,148,966 | Hebden   | Aug. 3, 1915   |
| 1,199,273 | Iljinsky | Sept. 26, 1916 |
| 1,431,136 | Villiger | Oct. 3, 1922   |
| 1,546,969 | Clavel   | July 21, 1925  |
| 1,716,720 | Ellis    | July 11, 1929  |
| 1,819,027 | Hood     | Aug. 18, 1931  |

FOREIGN PATENTS

| Number     | Country       | Date           |
|------------|---------------|----------------|
| 166,835    | Germany       | Jan. 12, 1906  |
| 213,266    | Great Britain | Jan. 1, 1906   |
| 15 340,267 | Great Britain | Dec. 19, 1930  |
| 419,061    | Germany       | Sept. 19, 1925 |

OTHER REFERENCES

- Matthews: Application of Dyestuffs, N. Y., 1920, 20 pages 413, 415, 428, 429, 430, 449.  
 Whittaker: Dyeing with Coal Tar Dyestuffs, 2nd ed., 1926, pages 122, 123, 129, 130, 132, 133, 140, 141.

**Certificate of Correction**

Patent No. 2,450,773.

October 5, 1948.

**EDWARD WEBER**

It is hereby certified that errors appear in the printed specification of the above numbered patent requiring correction as follows:

Column 2, line 50, for the words "which machine" read *winch machine*; column 3, lines 68 and 69, strike out "Serial No. 528,711, filed March 20, 1944, now abandoned" and insert instead *Serial No. 528,771, filed March 30, 1944, now Patent No. 2,420,729*; column 6, line 14, list of references cited, for "Jan. 1, 1906" read *Jan. 1, 1925*; and that the said Letters Patent should be read with these corrections therein that the same may conform to the record of the case in the Patent Office.

Signed and sealed this 5th day of April, A. D. 1949.

[~~initials~~]

**THOMAS F. MURPHY,**  
*Assistant Commissioner of Patents.*